

# United States Patent Office

3,033,796  
Patented May 8, 1962

1

3,033,796

ACID PICKLING BATH CONTAINING INHIBITOR  
AND METHOD OF TREATING FERROUS METALS  
Thomas W. Findley, La Grange, and Burton H. Robin  
and John E. Farbak, Chicago, Ill., assignors to Swift &  
Company, Chicago, Ill., a corporation of Illinois  
No Drawing. Filed Jan. 23, 1957, Ser. No. 635,585  
13 Claims. (Cl. 252—148)

The present invention relates to pickling methods and compositions and to corrosion and rust inhibiting materials and processes.

A dark coating of iron oxide (mill scale) forms on the surface of iron and steel during certain processing steps such as hot rolling and forging. This oxide film must be removed before the metal can be cold rolled, galvanized, tinned, electroplated, etc. In commercial operations mill scale is usually eliminated by pickling the iron or steel sheets, plates, bars, etc., in a suitable acid solution. In order to be acceptable, the acid pickling bath should be capable of casting off or dissolving the scale without unduly attacking the surface of the metal itself.

Although pickling is effective in removing mill scale, the acid treatment highly activates the surface of the treated metal, which immediately rusts on contact with oxygen. This rusting occurs as a "flash" reaction after the metal is water rinsed to free it from acid and while it is being air dried. Immediate rusting of this type is referred to as "sulling" or flash rusting and constitutes a serious problem in any industry where a rust-free metal is required.

Inasmuch as commercial pickling operations are often carried out under extreme conditions, materials added to a pickling bath to control corrosion, rust, etc., must be capable of performing at high acid concentrations and high temperature levels. Ordinarily, steel, for example, is pickled in a bath containing from about 10 percent to 25 percent  $H_2SO_4$  for about  $\frac{1}{2}$  minute to 5 minutes at a temperature of about  $75^\circ C$ . to about  $106^\circ C$ .

Another problem often encountered in pickling processes is the escape of acid fumes from the bath into the atmosphere. These fumes have long troubled steel producers. They constitute a hazard and are a source of discomfort to workers in the area of the pickling operations. In addition, the fumes tend to corrode nearby machinery and structures.

A continuing search has been carried out to find substances which, when added to acid pickling baths, acid scrubbers, and rinse baths, would lessen corrosion losses and would prevent "sulling" and the formation of harmful fumes. Although many additives have proved to be helpful for these purposes, none of the materials heretofore discovered have been entirely satisfactory.

It is, therefore, an object of the present invention to provide new pickling compositions and new pickling methods which protect metal surfaces against acid attack without diminishing the ability of the pickling bath to remove oxide film.

An additional object of the present invention is to provide pickling compositions and pickling methods which substantially eliminate flash rusting or "sulling."

A further object is to provide improved pickling compositions and pickling methods capable of removing oxide film without causing the evolution of harmful amounts of fumes from the pickling bath.

Another object of the present invention is to provide an improved iron and steel rinsing composition and method of rinsing iron and steel which substantially prevents immediate rusting.

A further object of the present invention is to pro-

2

vide a method of pickling iron and steel which prolongs the life of the acid bath.

Other objects and advantages of this invention will become apparent to those skilled in the art from the following detailed description.

Generally, the present invention comprises the discovery that conventional pickling, scrubbing, and rinse baths can be greatly improved by adding to said baths a member taken from the group having the following general formula:



where  $m$  is an integer from 0 to 19,  $n$  is an integer from 0 to 4,  $p$  is an integer from 0 to 19,  $y$  is an integer from 0 to 17 and  $m+2n+ny+3+p$  is an integer from 10 to 22; where at least one of  $W$  and  $X$  is selected from the group consisting of  $[-NR'R''H]^+[An]^-$ , and  $-NR'R'$ ; where  $W$  is selected from the group consisting of



and  $-NR'R''$  when  $X$  is selected from the group consisting of  $H$  and  $OH$ ; and where  $W$  is selected from the group consisting of  $[-NR'R''H]^+[An]^-$ ,  $-NR'R'$ ,  $H$  and  $OH$  when  $X$  is selected from the group consisting of  $[-NR'R''H]^+[An]^-$ , and  $-NR'R''$ ; and where  $R'$  is selected from the group consisting of alkyl and alkylool,  $R''$  is selected from the group consisting of  $H$ , alkyl and alkylool, where  $Z$  is selected from the group consisting of  $CH_2OH$ ,  $COOH$ ,  $CONR'R''$  and  $COOC_sH_{2s}NR''H$  where  $s$  is an integer from 2 to 8 and where  $[An]^-$  is an anion.

Pickling solutions containing widely divergent amounts of the above described ingredients have been found to be effective in inhibiting corrosion, controlling harmful fumes, substantially preventing flash rusting or "sulling," etc. Solutions having an inhibitor concentration of only 0.001 percent, for example, will improve the pickling operation, whereas satisfactory results can be obtained when as much as 25 percent or more of the ingredient is added to the baths. The effectiveness of the inhibiting compound does not evidence a sharp break when the concentration is changed. Although the amount of inhibitor added to the bath can vary extensively, it has been found that a concentration range of between about 0.01 percent and about 5.0 percent is preferred in most cases. Sulfuric acid is normally selected as the pickling acid in commercial operations. Other acids such as hydrochloric, phosphoric, and sulfamic, however, are likewise suitable.

The inhibitors of the present invention can be prepared by reacting a fatty material such as an epoxy, halogenated or haloxydrolated fatty acid, ester, amide, or alcohol having an alkyl chain length of from 10 to 22 carbon atoms with a primary or secondary alkylamine or alkyloolamine. Examples of compounds formed in the above reactions are: hydroxy alkylamino fatty acids and their esters and amides; hydroxy alkyloolamino fatty acids and their esters and amides; alkylamino fatty acids and their esters and amides; and alkyloolamino fatty acids and their esters and amides. The preparation of alkyloolamino fatty acids and their esters and amides is described in United States Patent No. 2,277,016. Hydroxy alkylamino fatty acids can be made as indicated in United States Patent No. 2,445,892. Methods of preparing hydroxy alkyloolamino fatty acids and their esters and amides and hydroxy alkyloolamino fatty alcohols are shown in copending United States Patent application Serial No. 629,235, filed December 19, 1956, and now U.S. Patent No. 2,993,919, under the name of "New Compositions of Matter."

The following examples show the use of the present invention in treating iron and steel products.

*Example I*

A pickling bath comparable to that used in the steel industry to remove mill scale was prepared by heating a 20 percent sulfuric acid solution to 95° C. Another bath was prepared in the same manner except that one (1) percent by weight of 9,10(10,9)diethanolaminohydroxystearic acid diethanolamide formed by condensing chlorohydroxystearic acid and diethanolamine was dissolved in the solution. Steel coupons cut from a steel sheet covered with mill scale were degreased and weighed and were then immersed in the pickling baths for 30 seconds, 5 minutes, and 30 minutes. The coupons were then rinsed in a water bath, allowed to air dry, and were again weighed. The following results were obtained:

|             |            |                                         |
|-------------|------------|-----------------------------------------|
| Control     | 30 seconds | Loss in weight= 49.3 g./m. <sup>2</sup> |
| 1% CHSA—DEA | 30 seconds | Loss in weight= 37.1 g./m. <sup>2</sup> |
| Control     | 5 minutes  | Loss in weight= 102 g./m. <sup>2</sup>  |
| 1% CHSA—DEA | 5 minutes  | Loss in weight= 41.3 g./m. <sup>2</sup> |
| Control     | 30 minutes | Loss in weight= 407 g./m. <sup>2</sup>  |
| 1% CHSA—DEA | 30 minutes | Loss in weight= 49.3 g./m. <sup>2</sup> |

Weight losses in the above chart and in the examples to follow are expressed in grams per square meter of coupon surface.

During the treatment, each of the control samples reacted vigorously with the acid, causing the evolution of considerable hydrogen gas. In contrast, coupons immersed in the baths containing the inhibitor reacted significantly less with the acid and very little hydrogen was given off. On being removed from the rinse bath and air dried, the control coupons rusted severely during drying, whereas the treated coupons remained shiny.

*Example II*

Two pickling baths containing 20 percent H<sub>2</sub>SO<sub>4</sub> were heated to 95° C. To one of the baths was added one (1) percent by weight of the reaction product of diethanolamine - methyldichloro - stearate, which is principally bis[N,N-bis (β-hydroxyethyl) amino] stearic acid diethanolamide. Steel coupons were pickled in each of the baths for 30 seconds, 5 minutes, and 30 minutes. The results of the treatment were as follows:

|             |            |                                         |
|-------------|------------|-----------------------------------------|
| Control     | 30 seconds | Loss in weight= 49.3 g./m. <sup>2</sup> |
| 1% MDCS—DEA | 30 seconds | Loss in weight= 40.5 g./m. <sup>2</sup> |
| Control     | 5 minutes  | Loss in weight= 102 g./m. <sup>2</sup>  |
| 1% MDCS—DEA | 5 minutes  | Loss in weight= 41.8 g./m. <sup>2</sup> |
| Control     | 30 minutes | Loss in weight= 407 g./m. <sup>2</sup>  |
| 1% MDCS—DEA | 30 minutes | Loss in weight= 46.1 g./m. <sup>2</sup> |

The coupons treated in the bath containing the inhibitor were found to be rust-free after the rinsing step, whereas coupons from the control bath rusted immediately on air-drying. The evolution of acid fumes was substantially eliminated in the MDCS—DEA bath.

*Example III*

Steel coupons were pickled for various lengths of time in a pickling bath prepared as shown in Example I except that the inhibitor was the diethanolamine condensate of methylpentachlorostearate, which is principally pentakis

[N,N-bis (β-hydroxyethyl) amino] stearic acid diethanolamide. The weight losses of the coupons were as follows:

|    |                                    |
|----|------------------------------------|
| 5  | 30 seconds—33.9 g./m. <sup>2</sup> |
| 10 | 5 minutes—42.3 g./m. <sup>2</sup>  |
| 15 | 30 minutes—44.3 g./m. <sup>2</sup> |

After the coupons were rinsed and air-dried, they were found to be rust-free. In addition, no acid fumes were observed to have evolved from the bath.

*Example IV*

Coupons were pickled in a bath, prepared as shown in Example I, which contained one (1) percent by weight of the diethanolamine condensate of alpha-bromostearic acid, which is principally α-[N,N-bis (β-hydroxyethyl) amino] stearic acid diethanolamide. The weight losses of the coupons were as follows:

|    |                                    |
|----|------------------------------------|
| 20 | 30 seconds—33.2 g./m. <sup>2</sup> |
| 25 | 5 minutes—40.5 g./m. <sup>2</sup>  |
| 30 | 30 minutes—46.1 g./m. <sup>2</sup> |

After the coupons were rinsed and air-dried, they were found to be rust-free. Again, no acid fumes were given off by the bath.

*Example V*

One (1) percent by weight of the diethanolamine condensate of alpha-bromomyristic acid, which is principally α-[N,N-bis (β-hydroxyethyl) amino] myristic acid diethanolamide, was added to a pickling bath as shown in Example I. After 30 minutes of treatment, a steel coupon was found to have lost 57.8 g./m.<sup>2</sup>. No fumes were given off from the bath and the coupon, after rinsing and air-drying was rust-free.

*Example VI*

Pickling baths containing the additives listed below were prepared as shown in Example I. Steel coupons immersed in the various baths did not evidence any "sulling" after the rinsing and drying steps. Each of the inhibitors effectively controlled metal corrosion and suppressed the evolution of acid fumes from the bath. The inhibitors, their concentrations, and pickling times were as follows:

|    | Inhibitor                                                                              | Concen-<br>tration,<br>percent | Pickling<br>Time, min. |
|----|----------------------------------------------------------------------------------------|--------------------------------|------------------------|
| 45 | 1,9,10(10,9) - butylethanolaminohydroxy - stearic acid butylethanolamide               | 1.0                            | 5                      |
| 50 | 2,9,10(10,9) - diisopropanolaminohydroxy - stearic acid diisopropanolamide             | 1.0                            | 5                      |
| 55 | 3. diethanolamine condensate of hypochlorinated soybean oil                            | 0.1                            | 5                      |
| 55 | 4. 9, 10 (10, 9)-monoethanolaminohydroxy - stearic acid monoethanolamide               | 0.1                            | 30                     |
| 55 | 5. reaction product of chlorohydroxystearic acid and 2-amino-2-methyl-1,3-propane-diol | 0.1                            | 5                      |
| 60 | 6,9,10(10,9) - diethanolaminohydroxyoctade - canol                                     | 0.1                            | 5                      |

*Example VII*

Ten (10) grams of 11-bromoundecylic acid was mixed with twenty (20) grams of dibutylamine and the mixture was refluxed for five hours. The product was not completely soluble in acid, an insoluble oil being present.

65 The soluble portion of the reaction mixture, principally 11-dibutylaminoundecanoic acid, was an effective corrosion inhibitor and anti-sulling agent for pickling of steel in 20 percent H<sub>2</sub>SO<sub>4</sub> at 95° C.

*Example VIII*

Twenty (20) grams of alpha-bromomyristic acid was mixed with 35 grams of dibutylamine and the mixture was refluxed for 5 hours. The product was not completely soluble in acid, an insoluble oil being present.

75 The soluble portion of the reaction mixture was an ef-

fective corrosion inhibitor and anti-sulling agent for pickling of steel in 20 percent  $H_2SO_4$  at 95° C.

*Example IX*

Forty-four (44) grams of dibromostearic acid was mixed with 63 grams of diethanolamine and the resulting solution was held at 180° C. for 1 hour. The product was soluble and surface-active in acid and water. It was an effective corrosion inhibitor and anti-sulling agent for pickling of steel in 20 percent  $H_2SO_4$  at 95° C.

*Example X*

Forty-four (44) grams of dibromostearic acid was mixed with 77 grams of dibutylamine and the resulting mixture was refluxed for 5 hours. The product was not completely soluble in acid, an insoluble oil being present. The soluble portion of the reaction mixture was an effective corrosion inhibitor and anti-sulling agent for pickling of steel in 20 percent  $H_2SO_4$  at 95° C.

*Example XI*

Fifty (50) grams of bromohydroxystearic acid was mixed with 68 grams of dibutylamine and the mixture was refluxed for 5 hours. The product was not completely soluble in acid, an insoluble oil being present. The soluble portion of the product was an effective corrosion inhibitor and anti-sulling agent for pickling of steel in 20 percent  $H_2SO_4$  at 95° C.

As is indicated above, the inhibitors of the subject invention are capable of functioning under extremely divergent conditions. In the following tests, pickling baths were prepared which consisted of 200 ml. of a particular acid containing an indicated amount of inhibitor (in these studies, the inhibitor was the condensation product of chlorohydroxystearc acid and diethanolamine). The corrosion inhibition capabilities of this inhibitor were tested by immersing previously pickled, rust-free steel coupons of known weight in the baths and then comparing their weight loss with the weight loss of coupons similarly treated in control baths. The acid baths were heated to 130° F., 170° F., and 200° F. Coupons were immersed in each of the baths for exactly 10 minutes, after which they were rinsed, dried, and weighed. The results of the tests were as follows:

CORROSION AT 130° F.

| Acid          | Inhibitor Conc. | Weight Loss, g./m. <sup>2</sup> | Percent Inhibition |
|---------------|-----------------|---------------------------------|--------------------|
| 2% $H_2SO_4$  | 0.00            | 1.05                            | 0                  |
|               | 0.01            | 0.450                           | 57.2               |
|               | 0.10            | 0.517                           | 50.8               |
|               | 1.00            | 0.417                           | 60.3               |
|               | 0.00            | 3.05                            | 0                  |
| 10% $H_2SO_4$ | 0.01            | 1.12                            | 63.3               |
|               | 0.10            | 0.567                           | 81.4               |
|               | 1.00            | 0.433                           | 85.8               |
|               | 0.00            | 4.54                            | 0                  |
|               | 0.01            | 2.45                            | 46.0               |
| 20% $H_2SO_4$ | 0.10            | 1.12                            | 75.3               |
|               | 1.00            | 0.433                           | 90.5               |
|               | 0.00            | 0.966                           | 0                  |
|               | 0.01            | 0.367                           | 62.0               |
|               | 1.00            | 0.385                           | 60.0               |
| 2% $H_3PO_4$  | 0.10            | 0.550                           | 43.0               |
|               | 1.00            | 0.550                           | 0                  |
|               | 0.00            | 1.45                            | 0                  |
|               | 0.01            | 0.550                           | 62.0               |
|               | 1.00            | 0.700                           | 51.7               |
| 10% $H_3PO_4$ | 0.01            | 0.550                           | 62.0               |
|               | 0.10            | 0.550                           | 63.2               |
|               | 1.00            | 0.550                           | 0                  |
|               | 0.00            | 2.28                            | 0                  |
|               | 0.01            | 0.917                           | 60.0               |
| 20% $H_3PO_4$ | 0.10            | 0.700                           | 69.3               |
|               | 1.00            | 0.417                           | 81.7               |
|               | 0.00            | 1.83                            | 0                  |
|               | 0.01            | 0.567                           | 69.0               |
|               | 1.00            | 0.433                           | 76.3               |
| 2% $HCl$      | 0.01            | 4.56                            | 0                  |
|               | 0.01            | 1.10                            | 76.0               |
|               | 0.10            | 0.833                           | 81.7               |
|               | 1.00            | 0.833                           | 81.7               |
|               | 0.00            | 35.5                            | 0                  |
| 10% $HCl$     | 0.01            | 5.67                            | 84.0               |
|               | 0.10            | 2.62                            | 92.6               |
|               | 1.00            | 2.10                            | 94.1               |

CORROSION AT 170° F.

|    |               |      |      |      |
|----|---------------|------|------|------|
| 5  | 2% $H_2SO_4$  | 0.00 | 5.67 | 0    |
|    |               | 0.01 | 1.73 | 70.0 |
|    |               | 0.10 | 1.40 | 75.3 |
|    |               | 1.00 | 0.92 | 83.7 |
|    |               | 0.00 | 17.6 | 0    |
| 10 | 10% $H_2SO_4$ | 0.01 | 5.80 | 67.0 |
|    |               | 0.10 | 2.95 | 83.3 |
|    |               | 1.00 | 1.33 | 92.5 |
|    |               | 0.00 | 34.8 | 0    |
|    |               | 0.01 | 14.9 | 57.3 |
|    |               | 0.10 | 6.70 | 80.8 |
|    |               | 1.00 | 2.20 | 93.7 |
|    |               | 0.00 | 4.03 | 0    |
|    | 2% $H_3PO_4$  | 0.01 | 1.28 | 68.3 |
|    |               | 0.10 | 1.17 | 71.0 |
|    |               | 1.00 | 1.77 | 56.0 |
|    |               | 0.00 | 9.24 | 0    |
| 15 | 10% $H_3PO_4$ | 0.01 | 3.00 | 67.5 |
|    |               | 0.10 | 1.60 | 82.7 |
|    |               | 1.00 | 1.80 | 80.5 |
|    |               | 0.00 | 13.9 | 0    |
|    | 20% $H_3PO_4$ | 0.01 | 6.10 | 56.2 |
|    |               | 0.10 | 2.75 | 80.2 |
|    |               | 1.00 | 2.08 | 85.1 |
|    |               | 0.00 | 8.02 | 0    |
| 20 | 2% $HCl$      | 0.01 | 1.37 | 82.9 |
|    |               | 0.10 | 1.02 | 87.3 |
|    |               | 1.00 | 0.93 | 88.4 |
|    |               | 0.00 | 41.0 | 0    |
|    | 10% $HCl$     | 0.01 | 7.80 | 81.0 |
|    |               | 0.10 | 3.26 | 92.1 |
|    |               | 1.00 | 2.77 | 93.3 |
| 25 | 20% $HCl$     | 0.00 | 178  | 0    |
|    |               | 0.01 | 86.0 | 51.7 |
|    |               | 0.10 | 27.4 | 84.6 |
|    |               | 1.00 | 14.9 | 91.6 |

CORROSION AT 200° F.

|    |               |      |      |      |
|----|---------------|------|------|------|
| 30 | 2% $H_2SO_4$  | 0.00 | 23.8 | 0    |
|    |               | 0.01 | 6.17 | 74.0 |
|    |               | 0.10 | 4.08 | 82.8 |
|    |               | 1.00 | 1.57 | 93.4 |
|    |               | 0.00 | 69.0 | 0    |
| 35 | 10% $H_2SO_4$ | 0.01 | 33.1 | 52.0 |
|    |               | 0.10 | 11.2 | 83.7 |
|    |               | 1.00 | 4.66 | 93.3 |
|    |               | 0.00 | 125  | 0    |
|    | 20% $H_2SO_4$ | 0.01 | 88.7 | 29.3 |
|    |               | 0.10 | 26.5 | 78.9 |
|    |               | 1.00 | 6.52 | 94.8 |
|    |               | 0.00 | 15.6 | 0    |
| 40 | 2% $H_3PO_4$  | 0.01 | 5.53 | 64.6 |
|    |               | 0.10 | 3.12 | 80.0 |
|    |               | 1.00 | 3.90 | 75.0 |
|    |               | 0.00 | 53.2 | 0    |
|    | 10% $H_3PO_4$ | 0.01 | 24.6 | 53.7 |
|    |               | 0.10 | 10.3 | 80.6 |
|    |               | 1.00 | 5.94 | 88.8 |
|    |               | 0.00 | 95.0 | 0    |
|    | 45            | 0.01 | 57.3 | 39.6 |
|    | 20% $H_3PO_4$ | 0.10 | 25.1 | 73.6 |
|    |               | 1.00 | 8.67 | 90.9 |
|    |               | 0.00 | 30.2 | 0    |
|    | 2% $HCl$      | 0.01 | 4.60 | 84.8 |
|    |               | 0.10 | 2.80 | 90.7 |
|    |               | 1.00 | 2.30 | 92.4 |
|    |               | 0.00 | 120  | 0    |
| 50 | 10% $HCl$     | 0.01 | 37.1 | 69.1 |
|    |               | 0.10 | 16.3 | 86.4 |
|    |               | 1.00 | 12.0 | 90.0 |
|    |               | 0.00 | 537  | 0    |
|    | 20% $HCl$     | 0.01 | 310  | 42.3 |
|    |               | 0.10 | 81.2 | 84.9 |
|    |               | 1.00 | 51.7 | 90.4 |

In commercial practice, steel is usually pickled in a 10-25 percent  $H_2SO_4$  solution heated to 75-100° C. to remove mill scale. Immediately after the steel is withdrawn from the pickling solution, it is thoroughly rinsed in a water bath to free it from acid. Unless an anti-sulling agent, such as the ingredients of the subject invention, has been added to the bath, the metal rusts as soon as it is dried after the rinsing step.

In the past, pickled but rusted ferrous products have been given a second and milder acid treatment (this is usually referred to as acid scrubbing) to remove the rust and brighten the surfaces of the metal. Unless the metal is thoroughly oiled as soon as it leaves the scrubber and subsequent water rinsing and drying zones, however, rust again forms. This immediate oiling has been found to be unnecessary when a minor amount of the anti-sulling agents of the present invention are added to the scrubber.

If it is desired, the anti-sulling properties of the subject inhibitors can be utilized by adding a minor amount

of the particular material to the water rinse bath. Concentration levels of from .01 percent to about 5 percent by weight of the inhibitor, for example, are satisfactory to prevent rinsed coupons from flash rusting.

The results of the foregoing tests illustrate certain of the outstanding characteristics of the iron and steel treating compositions of the present invention. There is, of course, substantial need in the steel industry for acid corrosion inhibitors which also possess anti-sulling properties. Steel treated with such materials does not require subsequent acid treatment and oiling, and can be electroplated, galvanized, etc., without further processing. Of almost equal importance to the industry is the fact that the present inhibitors control the escape of harmful acid fumes from the pickling baths. This beneficial property considerably improves working conditions around the bath and prevents acid vapors from corroding surround machinery. The present process and compositions have the further advantage of being fully amenable to established procedures inasmuch as the inhibitor is effective under almost any conditions and does not lengthen pickling time.

Of the compositions and methods described in the present invention, those that contain or make use of hydroxyalkylolamino compounds are especially effective. The unexpected success of these materials in particular probably is due at least in part to their unusual solubility characteristics.

An essential feature of the inhibitors of the present compositions is that they have either a primary or a secondary amine group substituted along an alkyl chain of a fatty acid or fatty acid derivative. Such derivatives include fatty esters, fatty amides, and fatty alcohols.

Obviously, many modifications and variations of the invention as hereinbefore set forth may be made without departing from the spirit and scope thereof, and therefore only such limitations should be imposed as are indicated in the appended claims.

We claim:

1. An acid bath for pickling ferrous metals containing about 2-25% acid and a minor amount sufficient to inhibit fumes of an inhibitor composition having the general formula:



where  $m$  is an integer from 0 to 19,  $n$  is an integer from 0 to 4,  $p$  is an integer from 0 to 19,  $y$  is an integer from 0 to 17; and  $m+2n+ny+3+p$  is an integer from 10 to 22; where at least one of  $W$  and  $X$  is selected from the group consisting of  $[-NR'R'H]^+[An]^-$ , and  $-NR'R''$ ; where  $W$  is selected from the group consisting of  $[-NR'R''H]^+[An]^-$ , and  $-NR'R''$  when  $X$  is selected from the group consisting of  $H$  and  $OH$ ; and where  $W$  is selected from the group consisting of  $[-NR'R'H]^+[An]^-$ ,  $-NR'R''$ ,  $H$  and  $OH$  when  $X$  is selected from the group consisting of



and  $-NR'R''$ ; and where  $R'$  is selected from the group consisting of alkyl and alkylol,  $R''$  is selected from the group consisting of  $H$ , alkyl and alkylol, where  $Z$  is selected from the group consisting of  $CH_2OH$ ,  $COOH$ ,  $CONR'R''$  and  $COOC_sH_{2s}NR''H$  where  $s$  is an integer from 2 to 8 and where  $[An]^-$  is an anion.

2. An acid bath for pickling ferrous metals containing about 2-25% acid and a small amount sufficient to inhibit acid fumes of 9,10(10,9) diethanolaminohydroxy stearic acid diethanolamide.

3. An acid bath for pickling ferrous metals containing about 2-25% acid and a small amount sufficient to inhibit fumes of bis [N,N-bis ( $\beta$ -hydroxyethyl) amino] stearic acid diethanolamide.

4. An acid bath for pickling ferrous metals containing about 2-25% acid and a small amount sufficient to inhibit

fumes of 9,10(10,9) butyl-ethanolaminohydroxy-stearic acid butylethanolamide.

5. An acid bath for pickling ferrous metals containing about 2-25% acid and a small amount sufficient to inhibit fumes of 9,10(10,9)-diisopropanolaminohydroxy stearic acid diisopropanolamide.

6. An acid bath for pickling ferrous metals containing about 2-25% acid and a small amount sufficient to inhibit fumes of  $\alpha$ -[N,N-bis( $\beta$ -hydroxyethyl)amino] myristic acid diethanolamide.

7. A method of treating ferrous metals which comprises: immersing said metals in an aqueous bath containing a small amount sufficient to inhibit sulling of a composition having the formula:



where  $m$  is an integer from 0 to 19,  $n$  is an integer from 0 to 4,  $p$  is an integer from 0 to 19,  $y$  is an integer from 0 to 17; and  $m+2n+ny+3+p$  is an integer from 10 to 22; where at least one of  $W$  and  $X$  is selected from the group consisting of  $[-NR'R'H]^+[An]^-$ , and  $-NR'R''$ ; where  $W$  is selected from the group consisting of  $[-NR'R''H]^+[An]^-$ , and  $-NR'R''$ , when  $X$  is selected from the group consisting of  $H$  and  $OH$ ; and where  $W$  is selected from the group consisting of



$-NR'R''$ ,  $H$  and  $OH$  when  $X$  is selected from the group consisting of  $[-NR'R''H]^+[An]^-$  and  $-NR'R''$ ; and where  $R'$  is selected from the group consisting of alkyl and alkylol,  $R''$  is selected from the group consisting of  $H$ , alkyl and alkylol, where  $Z$  is selected from the group consisting of  $CH_2OH$ ,  $COOH$ ,  $CONR'R''$  and  $COOC_sH_{2s}NR''H$  where  $s$  is an integer from 2 to 8 and where  $[An]^-$  is an anion.

8. In a process of conditioning ferrous metals wherein said metals are conditioned in an aqueous acid pickling bath the step which comprises immersing said metals in an aqueous bath containing a small amount sufficient to inhibit sulling of 9,10(10,9) diethanolaminohydroxy stearic acid diethanolamide.

9. In a process of conditioning ferrous metals wherein said metals are conditioned in an aqueous acid pickling bath the step which comprises immersing said metals in an aqueous bath containing a small amount sufficient to inhibit sulling of bis[N,N-bis( $\beta$ -hydroxyethyl)amino] stearic acid diethanolamide.

10. In a process of conditioning ferrous metals wherein said metals are conditioned in an aqueous acid pickling bath the step which comprises immersing said metals in an aqueous bath containing a small amount sufficient to inhibit sulling of 9,10(10,9) butyl-ethanolaminohydroxy stearic acid butylethanolamide.

11. In a process of conditioning ferrous metals wherein said metals are conditioned in an aqueous acid pickling bath the step which comprises immersing said metals in an aqueous bath containing a small amount sufficient to inhibit sulling of 9,10(10,9) diisopropanolaminohydroxy stearic acid diisopropanolamide.

12. In a process of conditioning ferrous metals wherein said metals are conditioned in an aqueous acid pickling bath the step which comprises immersing said metals in an aqueous bath containing a small amount sufficient to inhibit sulling of  $\alpha$ -[N,N-bis( $\beta$ -hydroxyethyl)amino] myristic acid diethanolamide.

13. The method of claim 7 wherein the aqueous bath is an acid pickling solution.

70 References Cited in the file of this patent

UNITED STATES PATENTS

1,766,902 Harrison \_\_\_\_\_ June 24, 1930  
1,810,946 Calcott et al. \_\_\_\_\_ June 23, 1931

(Other references on following page)

## UNITED STATES PATENTS

|           |                        |               |           |
|-----------|------------------------|---------------|-----------|
| 2,006,216 | Macarthur et al. ----- | June 25, 1935 | 2,807,585 |
| 2,080,553 | Wilson et al. -----    | May 18, 1937  | 2,831,814 |
| 2,277,016 | Guest -----            | Mar. 17, 1942 | 2,901,430 |
| 2,445,892 | Swern et al. -----     | July 27, 1948 | 2,902,447 |
| 2,564,749 | Bried -----            | Aug. 21, 1951 | 5         |
| 2,564,758 | Haggard -----          | Aug. 21, 1951 | 1,059,577 |
| 2,691,637 | Waibel -----           | Oct. 12, 1954 | 736,638   |
| 2,801,979 | Hager et al. -----     | Aug. 6, 1957  |           |

|                        |                |
|------------------------|----------------|
| Gardner et al. -----   | Sept. 24, 1957 |
| Chester et al. -----   | Apr. 22, 1958  |
| Chiddix et al. -----   | Aug. 25, 1959  |
| Gunderson et al. ----- | Sept. 1, 1959  |

## FOREIGN PATENTS

|                     |                |
|---------------------|----------------|
| France -----        | Nov. 10, 1953  |
| Great Britain ----- | Sept. 14, 1955 |